

Patented May 19, 1931

1,805,981

## UNITED STATES PATENT OFFICE

RICHARD BUCKMINSTER FULLER, OF LAWRENCE, NEW YORK, ASSIGNOR, BY MESNE  
ASSIGNMENTS, TO THE SOUNDEX CORPORATION, A CORPORATION OF ILLINOIS

## PROCESS OF MANUFACTURING FIBROUS BLOCKS

No Drawing. Original application filed December 31, 1924, Serial No. 758,991. Divided and this application filed March 1, 1927. Serial No. 171,908.

This application is a division of my earlier application, Ser. No. 758,991, filed December 31st, 1924, which has become Patent No. 1,634,900 and relates to certain phases of a 5 process of making fibrous blocks such, for example, as those described in Hewlett Patent No. 1,604,097, dated February 16, 1926.

In the manufacture of the blocks referred to, a particularly suitable fibrous material is 10 shredded wood fibre known as excelsior, but other fibrous material such as straw may be used. A suitable binder for use with such fibrous material is a mixture of magnesium oxide and magnesium chloride, while another 15 is slaked lime.

For the purposes of illustration I will describe my process in conjunction with the use of excelsior and a binder of magnesium oxide and magnesium chloride.

20 Excelsior is obtainable in compact bales. This may be broken up by hand and material then cut up into pieces of even length as by an ensilage cutter of standard design such as is used by farmers in cutting up fodder for 25 use in silos. As the excelsior at this stage is treated dry, some fire risk is attendant on this stage of the operations which may be advantageously conducted in a separate building.

30 The broken up excelsior is then conducted, preferably by the aid of an air current, to the mixing point where it is mixed with the binder which should be in substantially liquid form or solution. The binder may be either sprayed over the excelsior and stirred in or a surplus of binder may be used and the excelsior submerged in it.

35 As I am seeking to make blocks which are very light and have a very high proportion of connected air cavities, the excelsior which has been treated with the binder should have any surplus binder allowed to drain off and then should be submitted to some form of violent agitation which will break up compacted 45 masses leaving separate pieces of fibrous material coated with the binder but not leaving compacted masses of the material. This may be accomplished by blowing the treated fibres to a second ensilage cutter. The blowing will 50 accomplish part of the necessary breaking up,

and if any further agitation is necessary, this will be insured by the second cutting.

The material thus treated should be formed into masses of a desired shape by putting the material into a mold where the binder can 55 set. In forming such masses, care should be taken not to apply any more pressure than is necessary, for it is particularly important that the pressure should not be sufficient to compress the material into a compact state. 60 One way in which this molding may be conducted is by blowing the fibrous material into a perforated mold as is set forth in my said earlier application.

What I claim is:

1. The process of producing fibrous blocks, which comprises the steps of treating fibrous material with a binder in substantially liquid form, subjecting the treated fibrous material in the absence of surplus binder to 70 violent agitation whereby compacted masses of the fibrous material are broken up, forming the fibrous material into blocks without the use of substantial pressure and letting the binder set whereby light masses are obtained of a rigid structure comprising a very high 75 percentage of connected air spaces.

2. A process as defined in claim 1, in which an air current is used to agitate the fibrous material after the treatment with the binder. 80

3. A process as defined in claim 1, in which an excess of binder is used which is drained off prior to the agitation referred to.

4. The process of producing fibrous blocks, which comprises agitating fibrous material 85 in the presence of a liquid binder to break up compacted masses of the material and to leave the separate pieces of the fibrous material coated with the binder, and then forcing the treated material into a forming mold 90 to form the same into a desired shape, the amount of force used being insufficient to cause a compression of the material into a compact state.

5. The process of forming a fibrous block, which comprises coating long, thin fibers with a magnesium binder, agitating them to promiscuously intertwine the fibers together and to break up compacted masses, and forcing the coated fibers into a forming mold to 100

form the same into a desired shape, the amount of force used being insufficient to compress the material into a compact state.

6. The process of producing fibrous blocks,  
5 which comprises agitating fibrous material in  
the presence of a liquid binder to break up  
compacted masses of the material and to  
leave the separate pieces of the fibrous ma-  
terial coated with the binder, and then forc-  
10 ing the treated material into a desired shape,  
the amount of force used being insufficient  
to cause a compression of the material into a  
compact state.

7. The process of forming a fibrous block,  
15 which comprises coating long, thin fibers  
with a magnesium binder, agitating them to  
promiscuously intertwine the fibers together  
and to break up compacted masses, forcing the  
coated fibers into a desired shape, the amount  
20 of force used being insufficient to compress  
the material into a compact state, and per-  
mitting the shaped mass to set.

**RICHARD BUCKMINSTER FULLER.**

**25**

**30**

**35**

**40**

**45**

**50**

**55**

**60**

**65**